

# UNITED STATES PATENT OFFICE.

RADCLYFFE FURNESS, OF JENKINTOWN, PENNSYLVANIA, ASSIGNOR TO THE MID-VALE STEEL COMPANY, OF PHILADELPHIA, PENNSYLVANIA, A CORPORATION OF PENNSYLVANIA.

## HIGH-SPEED-TOOL-STEEL ALLOY.

1,233,862.

Specification of Letters Patent. Patented July 17, 1917.

No Drawing.

Application filed March 12, 1917. Serial No. 154,134.

To all whom it may concern:

Be it known that I, RADCLYFFE FURNESS, a citizen of the United States, residing at Jenkintown, county of Montgomery, and 5 State of Pennsylvania, have invented a new and useful Improvement in High-Speed-Tool-Steel Alloys, of which the following is a full, clear, and exact description.

The object of my invention is to produce 10 a new and improved high speed tool steel having a cutting efficiency superior to tool steels of an analogous character.

I have discovered that when to steel is added both cobalt and uranium, especially 15 when these are associated with tungsten, chromium and vanadium, a substantial increase in cutting efficiency is attained.

I prefer an alloy of steel containing about 4.5% of cobalt, about .7% of uranium, about 20 13.5% of tungsten, about 3.5% of chromium, and about 1.5% of vanadium. The carbon of the steel should constitute about .7% of the entire alloy. The steel may contain the usual proportions of manganese, phosphorous, 25 silicon and sulfur.

It is preferred to add the uranium in the crucible or in the ladle.

It is found that the addition of uranium, when cobalt also is added, improves the quality of the steel even though only a relatively 30 small proportion of the uranium actually added is found to remain in the finished product. Such an alloy, therefore, in which the percentage of uranium remaining in the 35 finished product is as low as .10% is within the scope of my invention, although the percentage of uranium may be increased to as much as 2%.

The cobalt may range between 3 and 7% 40 and the tungsten between 12 and 20%; although if, as is known, cobalt in part displaces the tungsten, the cobalt may be increased as high as 15 or 20%, while the tungsten may be reduced as low as 9%. The 45 chromium should be between 3 and 4%, although it may range from 2 to 6%. I add vanadium to obtain the well known qualities

which vanadium imparts to the alloy, if those qualities are desired, the amount ranging from .50 to 2 per cent. 50

The carbon may vary from .5 to .9 per cent.

Where in the claims I refer to the ordinary high speed tool steel additions, I mean to include one or more of those specified, 55 namely: tungsten, chromium and vanadium, or their known substantial equivalents.

It will be understood that the preferred proportion of uranium added is so small 60 that it cannot accurately be said to in part replace the known high speed tool steel additions, such as cobalt and tungsten, these being used in substantially the same proportions as heretofore, the addition of uranium, even in an apparently negligible proportion, 65 having been discovered by me to improve the cutting efficiency of high speed tool steels provided they contain cobalt.

Having now fully described my invention what I desire to claim and protect by Letters Patent is: 70

1. A high speed tool steel containing uranium, cobalt and the ordinary high speed tool steel additions.

2. A high speed tool-steel alloy containing 75 uranium, cobalt, tungsten and chromium.

3. A high speed tool-steel containing uranium, cobalt and tungsten.

4. A high speed tool-steel containing uranium .10 to 2%, cobalt 3 to 20% and the 80 ordinary high speed tool steel additions.

5. A high speed tool-steel containing uranium .10 to 2%, cobalt 3 to 20% and tungsten 9 to 20%.

6. A high speed tool-steel containing uranium .10 to 2%, cobalt 3 to 20%, tungsten 9 to 20% and chromium 2 to 6%. 85

In testimony of which invention, I have hereunto set my hand, at Philadelphia, on this 8th day of March, 1917.

RADCLYFFE FURNESS.

Witnesses:

JOSEPH ENTWISLE,  
HARRY D. SIEGFRIED.